

# United States Patent Office

2,791,815

Patented May 14, 1957

1

2,791,815

## RISER COMPOSITION AND A METHOD OF USING THE SAME

Harry Baldwin Kinnear, Columbus, Ohio, assignor, by mesne assignments, to Chromium Mining and Smelting Corporation, Limited, Sault Ste. Marie, Ontario, Canada, a corporation of Ontario

No Drawing. Application October 5, 1953,  
Serial No. 384,334

2 Claims. (Cl. 22—215)

This invention relates to a riser composition and to a method of using the same. More particularly, the invention relates to a riser composition for maintaining the risers of copper-base castings fluid for a period of time beyond which such risers would normally solidify whereby to substantially prevent pipe and to provide even shrinkage of the riser.

Heretofore, riser compositions for copper-base castings such as brass or bronze castings have generally included copper oxide, a reducing agent for the copper oxide and a fluxing material. These known riser compositions are exothermic and are ignited in contact with the molten riser of a copper-base casting to react with formation of metallic copper and a supernatant slag and with the evolution of considerable heat. The known exothermic compositions provide a layer of molten copper in contact with the top of the riser and do not contaminate the material of the riser with undesired metallic constituents such as iron. While such riser compositions are generally satisfactory, they are expensive.

An object of the present invention is to provide a riser composition for copper-base alloy castings that will maintain the riser fluid for an extended period of time without contamination of the riser. The compositions of the present invention do not necessarily include copper oxide as an ingredient and are composed of relatively inexpensive ingredients.

Another object of the invention is to provide a relatively inexpensive riser composition for copper-base castings that includes iron and yet does not contaminate the risers with any substantial quantity of iron.

Another object is to provide a process for maintaining the risers of copper-base castings fluid for an extended period of time by igniting in contact with the riser an iron-containing, exothermic composition that burns to form a slag containing substantially no metallic iron or only very small amounts of metallic iron as inclusions in the slag. Where metallic iron inclusions are present in the slag, they are largely out of contact with the copper alloy riser and hence do not add to the riser any substantial quantity of iron. It is important that the risers do not pick up iron because they are removed from the castings after solidification and are remelted with additional casting metal for reuse. Any substantial iron pick-up in the risers, gates or hot tops would result in an undesirably high iron analysis of casting metal in which such risers and the like are reused.

The exothermic riser compositions of the present invention include an intimate mixture of finely divided reducing agent, an oxidizing agent and a fluxing or slag-forming ingredient. Preferably ferrosilicon having a high silicon content is used as the reducing agent; although other reducing agents such as calcium silicide may be used. A silicon content of 90% or more is preferred.

Preferably, sodium nitrate is used as the oxidizing agent although other oxidizing agents such as potassium nitrate an alkali metal chlorate, an alkali metal perchlorate or manganese dioxide may be used. The oxidizing agent

2

normally is a solid material at ordinary room temperatures.

The slag-forming ingredient preferably is mill scale which is substantially  $Fe_3O_4$ . Other fluxing or slag-forming ingredients such as other oxides of iron or alumina may 5 also be employed to advantage either singly or in combination. The fluxing agent may be ferric oxide,  $Fe_2O_3$ .

The ingredients of the composition are so chosen and so proportioned as to liberate upon combustion a large 10 amount of heat that is sufficient to form a fluid slag that maintains the riser fluid for a substantial period of time. The composition of the slag formed is more or less a neutral sodium-iron silicate.

Sufficient oxidizing agent is incorporated in the composition to oxidize all of the silicon of the ferrosilicon to  $SiO_2$ . If insufficient oxidizing agent is used, the silicon of the ferrosilicon may reduce some of the fluxing material to yield metallic iron which must be kept at a minimum in the slag.

Where sodium nitrate is used as the oxidizing agent, the reaction is believed to proceed substantially in accordance with the following equation:

Equation No. 1.



The stoichiometric ratio of sodium nitrate to silicon in accordance with this reaction is about 2.45 parts of sodium nitrate by weight to each part by weight of silicon. However, the ratio of sodium nitrate to silicon may be 30 varied within reasonable limits and amounts ranging from about 2 parts of sodium nitrate to 3½ parts of sodium nitrate for each part of silicon can be used. Preferably, from 2-3 parts of sodium nitrate for each part of silicon are employed. Where mill scale is used as the fluxing material, sufficient mill scale is incorporated to form a neutral iron silicate slag with that part of the silica produced by the exothermic reaction that is not associated with the metal oxide residue of the oxidizing agent in a neutral alkali metal silicate.

As mentioned hereinbefore the components of the exothermic mixture are preferably so chosen that the resulting slag will be a substantially neutral one. The metal oxide fraction of the oxidizing agent enters the slag as a neutral silicate. For example, where sodium nitrate is 40 the oxidizer, two molecules of  $Na_2O$  combine with one molecule of  $SiO_2$  to provide neutral sodium silicate of the formula  $Na_4SiO_4$ . Referring to Equation No. 1 hereinbefore it will be seen that for each two molecules of  $Na_2O$  produced, five molecules of  $SiO_2$  are concurrently 45 yielded. Since the two molecules of  $Na_2O$  combine with one molecule of  $SiO_2$ , it will be seen that four molecules of  $SiO_2$  are in excess of the amount required for a neutral slag. A fluxing material is added to the ingredients of the exothermic reaction mixture to satisfy the requirements 50 of the excess silica to form a neutral slag. Thus, where mill scale is used as a fluxing agent, four molecules of  $Fe_3O_4$  in the form of mill scale are included for each five molecules of silicon and four molecules of sodium nitrate in the reaction mixture. The four molecules of  $Fe_3O_4$  combine with the four molecules excess of  $SiO_2$  resulting from the exothermic reaction to provide a neutral iron silicate slag of the composition  $Fe_3SiO_6$ . The reaction thus may be summarized in the following equation:

Equation No. 2



The amount of fluxing agent may vary somewhat from that required to yield a neutral silicate slag. The resulting 70 slag may be either acid or basic within reasonable limits. For example, for each five molecules of Si and four molecules of sodium nitrate in the reaction mixture, from two

to eight molecules of  $Fe_3O_4$  may be incorporated in the reaction mixture. The employment of other fluxing agents such as alumina is governed by similar principles. In accordance with Equation No. 2, each part by weight of silicon requires 2.45 parts by weight of sodium nitrate and 6.6 parts by weight of  $Fe_3O_4$ . For each part by weight of silicon the sodium nitrate may fall within the range of 2 to 3½ parts by weight and the  $Fe_3O_4$  may fall within the range 3 to 12 parts by weight.

Riser compositions in accordance with the invention are in the form of an intimate mixture of finely divided materials. The compositions may be employed as mixtures of powdered ingredients or the powdered ingredients preferably are formed into agglomerates or briquettes. If agglomerates are desired, it is beneficial to employ a binder. The oxidizing agent itself may form the binder or an auxiliary binding material may be added to the powdered mixture and the mixture thereafter formed into agglomerates. Binders such as molasses water, waste sulfite liquor or inorganic binders such as sodium silicate may be used. Conventional methods are employed to form agglomerates such as pressing or rolling the powder into balls. Agglomerates approximating spheres having diameters from ¼" to ½" are especially suitable but the size and shape of the agglomerates may vary.

In use, the riser compositions of the invention are placed upon the top of a molten riser of a copper-base alloy casting immediately after pouring and while the riser is still fluid. The heat of the molten metal in the riser ignites the composition of the invention which burns with the evolution of large amounts of heat. The slag formed by the self-contained combustion of the material is fluid and remains hot for a sufficiently long time to insure proper feeding of the casting from the riser during solidification of the casting. Any metallic iron that remains from the ferrosilicon of the composition tends to agglomerate into minute shot-like particles that remain suspended in the slag and do not come in contact with the metal of the riser. It is highly desirable and very important that the ferrosilicon be of a high silicon grade in order that residual iron be kept at a minimum. Ferrosilicon having at least 90% silicon and preferably having 95% silicon is preferred. Ferrosilicon metal of 98% or greater purity may be used in whole or in part.

After the copper-base casting has solidified, the frozen slag resulting from treatment of the riser in accordance with the present invention is readily and cleanly broken away from the riser and discarded. The riser is separated from the casting in the usual manner. The risers treated by the compositions of the present invention show practically no iron pick-up and are essentially of the same composition as the original copper-base alloy. These risers are clean and can be re-melted for further casting operations.

The following table illustrates the iron pick-up in risers per application of a typical riser composition (Mill scale 65 parts, sodium nitrate 24 parts, and ferrosilicon—95% Si—11 parts by weight), the maximum iron build up where each melt subsequent to the first contains 40% of risers

from a previous cast to which the riser composition of the invention is applied and a comparison of these values with ASTM specifications for maximum iron content.

TABLE I

| Type of Copper-Base Alloy                              | Iron Pick Up per Application of Riser Composition, percent | Maximum Iron Build Up with 40% of Riser in Each Melt, percent | Maximum Iron Content; A. S. T. M. Specifications, percent |
|--------------------------------------------------------|------------------------------------------------------------|---------------------------------------------------------------|-----------------------------------------------------------|
| (1) Leaded Red Brass: 85 Cu, 5 Sn, 5 Pb, 5 Zn.....     | 0.01-0.03                                                  | 0.017-0.05                                                    | 0.30                                                      |
| (2) Yellow Brass: 60 Cu, 40 Zn.....                    | 0.06-0.15                                                  | 0.10-0.25                                                     | 0.60-0.75                                                 |
| (3) Leaded Tin Bronze: 87 Cu, 8 Sn, 1 Pb, 4 Zn.....    | 0.01-0.05                                                  | 0.017-0.084                                                   | 0.15-0.25                                                 |
| (4) Manganese Bronze (High Strength Yellow Brass)..... | 0.11                                                       | 0.18                                                          | 2.0-3.0                                                   |
| (5) Aluminum Bronze.....                               | 0.03                                                       | 0.05                                                          | 2.5-5.0                                                   |

From the foregoing table it is seen that where riser compositions of the present invention are employed the iron pick-up in risers per application of the riser composition of the invention is negligible and the maximum iron build up where 40% of risers are reused in subsequent melts is far below maximum ASTM specifications.

The invention will be illustrated and described with greater particularity in the following detailed examples.

#### Example I

30 Mill scale and ferrosilicon (95% Si) are separately ground in a ball mill to finenesses of about 55-65% through a 200 mesh screen and all of the material through a 100 mesh screen. The sodium nitrate is employed in a fine, granular condition substantially all through a 100 mesh screen.

To 500 lbs. of ground mill scale are added 85 lbs. of ground ferrosilicon and 185 lbs. of granular sodium nitrate. These powders are thoroughly mixed and to the mixture is added 31 lbs. of molasses water containing 8

40 lbs. of black strap molasses and 23 lbs. of water as a binder. The mixture is tumbled in a rotary mixer to form nodules ranging in size from ¼" to ½" in diameter. As the nodules are formed they are removed from the tumbling mixture. The green nodules are dried in an oven at 110°.

45 C. until the moisture content is less than about 1%. The nodules as dried are ready for use in treating risers of copper-base castings.

Sufficient of the riser compound is employed to provide from ½ to ¾" of slag on the riser. The mixture is ignited on the top of a riser of a freshly poured yellow brass casting. The mixture ignites readily from the heat of the riser and burns rapidly. The slag produced by the riser composition is broken and examined after freezing and only a few tiny beads of metal are found dispersed in the slag. The brass casting is sound and the riser is flat on top and has no pipe.

55 Table II hereinafter shows the composition of additional riser mixtures in accordance with the invention. The procedures for making and using the mixtures are similar to those described in Example I.

TABLE II

| Mix    | Composition, percent |          |                       |               |             | Ratio, $NaNO_3$ : $FeSi$ | Ratio, Mill Scale: $NaNO_3$ + $FeSi$ | Approx. Temp. of Slag, °F |
|--------|----------------------|----------|-----------------------|---------------|-------------|--------------------------|--------------------------------------|---------------------------|
|        | Mill Scale           | $NaNO_3$ | $FeSi$ , 90-95% Grade | Silicon Metal | Other       |                          |                                      |                           |
| 1..... | 53.4                 | 33.3     | —                     | 13.3          | —           | 2.5                      | 1.14                                 | 2,900                     |
| 2..... | 64.0                 | 23.6     | 10.4                  | —             | $MnO_2$ 2.0 | 2.47                     | 1.98                                 | 2,875                     |
| 3..... | 65.0                 | 24.0     | 11.0                  | —             | —           | 2.18                     | 1.86                                 | 2,800                     |

Each of the mixtures of Table II ignites readily and burns rapidly. Only a few tiny beads of metal are found in the slags resulting from combustion of the mixes.

I claim:

1. An exothermic riser composition for providing a hot top on the risers of copper-containing castings to prevent pipe consisting essentially of ferrosilicon containing more than 90% silicon, sodium nitrate and mill scale in the substantial molecular ratio of 5 molecules of silicon to 4 molecules of sodium nitrate to 4 molecules of  $Fe_3O_4$ . 10

2. A process for maintaining the risers of copper-containing castings fluid to prevent pipe which comprises igniting in contact with the top of a molten riser of a copper-containing casting an exothermic riser composition consisting essentially of an intimate mixture of finely divided ferrosilicon containing more than about 90% silicon,

sodium nitrate and mill scale in the substantial molecular ratio of 5 molecules of silicon to 4 molecules of sodium nitrate to 4 molecules of  $Fe_3O_4$ .

References Cited in the file of this patent

UNITED STATES PATENTS

2,280,872 Udy ----- Apr. 28, 1942  
2,513,602 Udy ----- July 4, 1950

FOREIGN PATENTS

673,605 Great Britain ----- June 11, 1952

OTHER REFERENCES

Metallurgy of Copper, by Newton-Wilson (1942 edition), pages 120 and 121 relied on.